



US007351512B2

(12) **United States Patent**  
Tan et al.

(10) Patent No.: US 7,351,512 B2  
(45) Date of Patent: Apr. 1, 2008

- (54) **OVERCOAT FOR A POLYMER SLEEVE MEMBER FOR A BLANKET CYLINDER AND A METHOD FOR MAKING THE OVERCOAT**

(75) Inventors: **Biao Tan**, Penfield, NY (US); **Craig M. Cody**, Scottsville, NY (US); **Po-Jen Shih**, Webster, NY (US); **Joseph A. Pavlisko**, Pittsford, NY (US)

(73) Assignee: **Eastman Kodak Company**, Rochester, NY (US)

(\*) Notice: Subject to any disclaimer, the term of this patent is extended or adjusted under 35 U.S.C. 154(b) by 504 days.

(21) Appl. No.: **11/017,486**

(22) Filed: **Dec. 20, 2004**

(65) **Prior Publication Data**  
US 2005/0143241 A1 Jun. 30, 2005

**Related U.S. Application Data**

(60) Provisional application No. 60/532,195, filed on Dec. 23, 2003.

- (51) **Int. Cl.**  
**G03G 21/00** (2006.01)  
(52) **U.S. Cl.** ..... 430/125.32; 492/56; 428/423.1;  
428/424.2; 428/447  
(58) **Field of Classification Search** ..... 430/125.32;  
492/56; 428/423.1, 424.2, 447  
See application file for complete search history.

(56) **References Cited**

## U.S. PATENT DOCUMENTS

- 5,337,129 A \* 8/1994 Badesha ..... 399/308

\* cited by examiner

*Primary Examiner*—Mark A. Chapman  
(74) *Attorney, Agent, or Firm*—Carl F. Ruoff

## ABSTRACT

This invention relates to a polymer sleeve including a polymer sidewall and a ceramer outer coating and a method for producing the polymer sleeve for use with a blanket cylinder in an electrophotographic process.

**19 Claims, 4 Drawing Sheets**





FIG. 1



*FIG. 2*  
(*PRIOR ART*)



*FIG. 3*  
(*PRIOR ART*)



FIG. 4



FIG. 5



FIG. 6

## 1

**OVERCOAT FOR A POLYMER SLEEVE  
MEMBER FOR A BLANKET CYLINDER AND  
A METHOD FOR MAKING THE OVERCOAT**

CROSS REFERENCE TO RELATED  
APPLICATION

Reference is made to and priority claimed from U.S. Provisional Application Ser. No. 60/532,195, filed Dec. 23, 2003, entitled OVERCOAT FOR A POLYMER SLEEVE MEMBER FOR A BLANKET CYLINDER AND A METHOD FOR MAKING THE OVERCOAT.

FIELD OF THE INVENTION

This invention relates to a method for producing a polymer sleeve for use with a blanket cylinder in an electrophotographic process wherein the polymer sleeve requires no metal core and includes a closely controlled external coating.

BACKGROUND OF THE INVENTION

In electrophotographic processes requiring an image cylinder and a blanket cylinder to produce electrophotographic copies, the image cylinder typically receives a charge, an image and a toner coating on the image area and then transfers the toner image to a blanket cylinder. The blanket cylinder transfers the toner image to a substrate, such as paper or the like, which passes via a web between the blanket cylinder and a back pressure roller to transfer the toner image to the substrate with the substrate thereafter being fused, as well known to the art.

In such processes, the blanket cylinder is a cylinder that typically includes a mandrel, which may be of aluminum, steel or any other suitably durable metal or conductive polymer of a suitable thickness to produce a noncompliant member that may be about 10 millimeters (mm) in thickness. The mandrel may include reinforcing structure internally and includes a very smooth, low out-of-round tolerance exterior. The blanket cylinder includes a mandrel and a sleeve positioned over the outside of the mandrel and is used for transfer of the images from the blanket cylinder to a substrate. The mandrel also includes fittings connected to each of its ends for positioning it in an electrophotographic copying machine and has an air inlet into an interior of the mandrel for an air discharge through a plurality of holes placed around one end of the mandrel near a tapered end of the mandrel.

The sleeves have been produced by use of a metal core, which is typically a noncompliant metal member, such as nickel or the like, which is produced by plating. The core must be seamless and must provide a very low variation surface outer diameter. The polymer layer has been positioned around the outside of the metal core, the metal core is mounted on a mandrel or the like, and the polymer layer is machined to a desired thickness. Additional exterior coatings have been applied by techniques such as ring coating and the like. The completed sleeve will have an internal diameter slightly less (typically about 100 microns) than the outer diameter of the mandrel upon which it is to be placed. This interference fit allows the sleeve to be firmly positioned on the outside of the mandrel after it is installed. The sleeve must have a smooth exterior and a closely controlled wall thickness.

The sleeve is typically installed by urging it toward and onto the tapered end section of the mandrel while air is

## 2

ejected through the holes at the end of the mandrel near the tapered section. The air injection permits the positioning of the sleeve on the mandrel by an air bearing technique as known to those skilled in the art. The interference fit between the sleeve and the mandrel is accomplished and the sleeve is retained snugly and firmly in position on the outside of the mandrel. The outside of the mandrel, including the sleeve, must have an outside diameter variation within a range of about +/-12.5 microns. This close tolerance is necessary to ensure accurate receipt of images from the image cylinder and accurate transmission of the images to the substrate by the blanket cylinder.

There are various other specific requirements for the blanket cylinder and it has been previously considered necessary to meet these other requirements as well as those discussed above by the use of a metal core in the sleeve. This is a relatively expensive, time-consuming step and the cores are relatively expensive. As a result, a continued effort has been directed to the development of methods for producing sleeves more economically that will meet the demanding requirements for the blanket cylinder sleeves.

SUMMARY OF THE INVENTION

According to the present invention, a method is provided for producing a sleeve for mounting on a mandrel to form a blanket cylinder for use in an electrophotographic process, the method provides producing a sleeve having a sidewall of a polymer selected from the group consisting of thermoplastic, thermoset and elastomeric polymers and rigid polyurethanes, the sleeve having an inner diameter from about 1 to about 20 percent less than the outer diameter of the mandrel and, coating the sleeve with an outer coating comprising a ceramer containing a polyurethane and tetraethoxyorthosilicate, the polyurethane having a molecular weight from about 20,000 to about 80,000 with the polyurethane and the tetraethoxyorthosilicate being present in a weight ratio from about 1.8 to about 2.3.

The invention further provides an improvement in a method for producing a sleeve for use on a mandrel to produce a blanket cylinder for use in an electrophotographic process, the sleeve consisting essentially of a sleeve of a polymer selected from the group consisting of thermoplastic, thermoset, and elastomeric polymers and rigid polyurethanes blends thereof and a ceramer coating comprising a polyurethane and tetraethoxyorthosilicate, the sleeve having an inner diameter from about 1 to about 20 percent less than the outer diameter of the mandrel, the improvement comprising adjusting the molecular weight of the polyurethane to from about 20,000 to about 80,000 and adjusting the weight ratio of the polyurethane and the tetraethoxyorthosilicate to from about 1.8 to about 2.3.

The invention also provides a sleeve adapted to fit over a mandrel to form a blanket cylinder for use in an electrophotographic process, the sleeve having a sidewall of a polymer selected from the group consisting of thermoplastic, thermoset and elastomeric polymers, polyurethanes and blends thereof, the sleeve having an inner diameter from about 1 to about 20 percent less than the outer diameter of the mandrel and, an outer coating comprising a ceramer containing a polyurethane and tetraethoxyorthosilicate, the polyurethane having a molecular weight from about 20,000 to about 80,000 with the polyurethane and the tetraethoxyorthosilicate being present in a weight ratio from about 1.8 to about 2.3.

## BRIEF DESCRIPTION OF THE DRAWINGS

FIG. 1 shows an embodiment of a process and system wherein a blanket cylinder according to present invention is used;

FIG. 2 is a schematic diagram of a mandrel and a sleeve, with the sleeve being positioned for installation on the mandrel;

FIG. 3 is a schematic diagram of a sleeve positioned on the mandrel;

FIG. 4 is a schematic diagram of a mold positioned for rotation and injection of polymer material to form a polymer sleeve according to the present invention;

FIG. 5 shows a mold body that has been coated by a ring coating process; and

FIG. 6 shows an apparatus for producing a polymer sleeve having an exterior coating and a polymer layer positioned in a mold.

## DESCRIPTION OF PREFERRED EMBODIMENTS

In the description of the figures, the same numbers will be used to refer to the same or similar components throughout in the discussion of the figures.

In FIG. 1, an electrophotographic process and system 10 are shown. The process includes an image cylinder 12 positioned in engagement with a blanket cylinder 14, which is positioned in engagement with a web 16 and a back pressure roller 18. A substrate 20, which may be paper or the like, is passed along a web 16 between blanket cylinder 14 and back pressure roller 18. The substrate, now bearing an image, is passed along web 16 to a fuser section 26 where it is fused as known to those skilled in the art. The direction of travel of the substrate is shown by arrow 22. A sensor 24 is positioned to ensure that substrate 20 passes in contact with blanket cylinder 14 at a proper time so that the image is properly positioned on substrate 20.

In the operation of the process, image cylinder 12 rotates in a direction shown by arrow 36 and blanket cylinder 14 rotates in a direction shown by arrow 42. Back pressure roller 18 turns in a direction as shown by arrow 19. A nip 38 is formed between image cylinder 12 and blanket cylinder 14. The nip is typically about 4.5+/-1 mm in width. Similarly, a nip 44 is formed between blanket cylinder 14 and back pressure roller 18. This nip is about 4 to about 10 mm in width. A cleaning station 28 is positioned to contact the surface of image cylinder 12 after it passes nip 38. The clean image cylinder surface then passes a charger station 30, a writer station 32 where an electrostatic image is placed on the surface of cylinder 12 and a toner section 34 that applies toner to the electrostatic image, which is then transferred at nip 38 to blanket cylinder 14. Blanket cylinder 14 transfers the image to substrate 20 and is thereafter cleaned by a cleaner 40 to ensure that a clean surface is provided on blanket cylinder 14 for transfer of an additional image from image cylinder 12.

As shown in FIG. 2, blanket cylinder 14 includes a mandrel 50 that has side walls 54 and ends 52 and includes a tube 60 which supports a bearing 62 in operative engagement with one end of mandrel 50 and a shaft 64 which supports a second bearing 66 in operative engagement with the other end of mandrel 50.

Tube 60 is adapted for the injection of air into mandrel 50, which includes near one of its ends, a taper 56, and a plurality of air holes 58. These air holes are used for the ejection of air during the installation of a sleeve over

mandrel 50. Mandrel 50 has an outside diameter 68, which is somewhat larger than the inner diameter 72 of a sleeve 70. Sleeve 70 as shown, is a polymer sleeve according to the present invention. Its end 74 is urged into engagement with tapered section 56 of mandrel 50 and the sleeve is placed over an outside diameter 68 of mandrel 50 by an air step process using the ejection of air through holes 58.

In FIG. 3, an installed sleeve, according to the present invention, is shown on mandrel 50. The mandrel and sleeve 10 that comprise blanket cylinder 14 are now assembled.

The blanket cylinder may have an outer diameter from about 40 mm to about 600 mm. While the diameter may vary widely, the variations in diameter or the out of round run out must be limited to +/-12.5 microns. This is necessary to 15 ensure that the proper nip is achieved between the blanket cylinder and the pressure roller and that good image transfer from the image cylinder to the blanket cylinder and from the blanket cylinder to the substrate is accomplished.

Desirably the outside of blanket cylinder sleeve 70 has a 20 Shore A hardness of about 65+/-5. The hardness is readily varied by changing the formulation of the polymer, as well known to those skilled in the art. The thickness of the sleeve wall is polymer and is rigid enough to handle. Further the 25 polymer desirably has a conductivity of at least  $10^7$  to  $10^{14}$  ohms·cm. Generally the conductivity of the blanket cylinder sleeve is less than for the image cylinder sleeve, although the charge on the blanket cylinder is typically higher than that on the image cylinder. To produce an acceptable exterior 30 surface on blanket cylinder 14, it is necessary that the wall thickness of the sleeve be held to a thickness variation of +/-12 microns. Generally the blanket cylinder sleeve exterior is more compliant than the exterior of the image cylinder sleeve.

Sleeves have been formed in the past by positioning the sleeves on a seamless metal core typically formed by plating. The metal core provided support for the positioning of the polymer around the metal core and then the polymer was machined to the required size. Both the requirement for 40 the metal core and the requirement for machining represent expensive and time consuming operations that have been required to achieve the precision necessary to produce the sleeves for the blanket cylinder.

As well known to those skilled in the art, a thin hard 45 release layer such as a sol-gel, a ceramer or a fluoropolymer may be placed on the outside of the sleeve for the blanket cylinder. This layer has been applied by processes such as ring coating, dipping and the like. It is also known that inorganic or organic layers may be applied over the outside 50 of the sleeve to modify surface properties such as surface energy. The use and application of such outer layers is not considered to constitute part of the present invention, which is directed to the production of a sleeve for a blanket cylinder meeting the exacting requirements for such a 55 sleeve.

According to the present invention, such sleeves are readily produced by a method providing positioning a quantity of polymer precursors, a suitable liquid polymer, or a liquefiable polymer in a mold with the mold then being 60 heated by a heater 90 to a suitable temperature to result in the presence of the polymer in the mold in a liquid form. A suitable mold is shown schematically in FIG. 4. The mold has a wall 78 and ends 82. Openings 84 are generally left in the ends. While the polymer could be introduced in a number 65 of ways, it is shown as being introduced through a tube 86 that supplies a quantity of polymer suitable to form a sleeve of the desired thickness and of uniform thickness in the

mold. The uniformity is achieved by spinning the mold while the polymer is heated and as the polymer moves through a molten phase. The molding may be done with a thermoplastic material, which after liquefying is allowed to cool back into a hardened phase. In any event, the formation of the solid sleeve is accomplished with rotation of the mold at a rate sufficient to produce a centrifugal force equal to at least five and preferably at least about 10 and desirably from about 5 to about 100 times the force of gravity at the inside of the mold until the polymer has solidified.

Suitable polymers comprise thermoplastic, thermoset and elastomeric polymers and particularly polyurethanes are preferred. With polyurethanes, polymer precursors may be placed into the mold and allowed to polymerize, cross-link and otherwise react to form the desired polymers as the mold spins. In any event, it has been found that when the inside of the mold is formed to have a surface within the required variations for the outside of the sleeve, that the inside of the sleeve and the sleeve wall thickness can be produced to sufficiently close tolerances by this method to enable its positioning over a mandrel and use on the blanket cylinder. Blends of the polymers may be used.

Typically the wall of the sleeve is at least partially comprised of thermoplastic, thermoset and elastomeric polymers or combinations thereof and particularly polyurethanes are preferred. Polysiloxanes and fluorocarbon polymers and copolymers may also be used. The properties of the polymer may be varied as known to those skilled in the art to produce the desired properties in the sleeve. The polymer may contain additives, fillers and the like as known to the art and may be used a blends of a plurality of polymers.

The heating and cooling of the mold may be at rates deemed suitable for the particular polymer used and desirably the rotation of the mold is continued until the polymer has reached a temperature of about 100° C. and thereafter until the polymer is cooled to a temperature selected for convenience in handling and the like. After cooling the sleeve typically releases from the inside of the mold by contraction of the polymer so that the sleeve is readily removed from the mold by simply removing one of ends 82 and removing the sleeve. The sleeve is then ready for use or for coating with additional materials that may be desired on its exterior. A heater 90 is shown but it will be understood that any suitable type of heater can be used.

While sleeves can be produced by the molding process described above, the sleeves can also be produced by use of a production mandrel with the sleeve being formed of a suitable polymer material positioned on the production mandrel with the production mandrel them being rotated to machine the polymer material to a desired configuration and thickness on the production mandrel. The sleeve is then removed from the production mandrel and can be used without a core. The polymer material can be placed on the production mandrel by any of a variety of known methods such as extrusion casting, injection casting, ribbon casting and the like, but in all instances the production mandrel must have an outer diameter smaller than the outer diameter of the mandrel. The sleeve has an inner diameter equal to the outer diameter of the production mandrel.

In either case, the use of the sleeve without the nickel core achieves certain advantages. Particularly, the nickel cores used in the sleeves for the blanket cylinder must be formed very precisely at a high cost. In addition, the handling of the nickel sleeve during the manufacturing process is high due to the intensive cleaning and priming steps required. Elimination of the use of a nickel core represents a substantial cost savings.

While the sleeve of the present invention may be formed by either process, they still require the positioning of an outer coating such as a ceramer, a sol-gel or a fluorocarbon polymer or copolymer on the exterior of the sleeve. As indicated previously, such coatings can be applied readily by ring coating, dipping and the like. If the molding process is used, the exterior coating may be applied as a layer either inside the mold prior to positioning the polymer body of the sleeve or as one constituent of the mixture placed in the 10 mold prior to rotation.

By the process of the present invention, sleeves for the blanket cylinder can be produced much more economically and more efficiently than with previously used methods. The sleeves produced are a polymer sleeve for use by positioning 15 it over an outer diameter of a mandrel. The polymer sleeve has a wall thickness from about 1 to about 20 mm, an inner diameter smaller than the outer diameter of the mandrel, a Shore A hardness of about 65+/-5 and a wall thickness variation of no more than about +/-12 microns from the 20 average wall thickness. These sleeves are highly desirable as replacement sleeves around the outside of mandrels in blanket cylinders. These sleeves are also much more economically produced while providing sleeves of an equivalent or superior quality to those produced by prior art 25 methods.

While the sleeves produced by the method described are beneficial because they are more economical and provide adequately controlled wall thicknesses and surface properties, they must be produced at a size somewhat less than the 30 outer diameter of the mandrel upon which they are to be placed. The undersizing is greater than that typically used with sleeves that contain a nickel core. As a result there is a tendency for the exterior coating on the sleeves to crack, wrinkle, or otherwise deform as a result of the positioning of 35 the sleeve over the mandrel. This cracking, wrinkling or deformation creates undesirable and unacceptable irregularities in the surface of the sleeve. Accordingly, considerable effort has been directed to developing sleeves and exterior coatings that do not suffer these shortcomings.

According to the present invention, such shortcomings are 40 avoided in sleeves that have an inner diameter from about 1 to about 20 and preferably from about 4 to about 12 percent less than the outer diameter of the mandrel. These sleeves are typically coated with an outer coating that may include 45 a ceramer containing a polyurethane and a tetraethoxyorthosilicate. A suitable tetraethoxyorthosilicate (TEOS) is available from Huls America, Inc.

These materials are typically used to produce a ceramer 50 coating that is placed on the outside of the sleeve. The ceramer coating desirably contains polyurethane having a molecular weight from about 20,000 to about 80,000 with the polyurethane and the tetraethoxyorthosilicate being present in the ceramer in a weight ratio from about 1.8 to about 2.3.

55 Preferably, the molecular weight is from about 30,000 to about 50,000 and with a diameter difference of from about 4 to about 12 percent, the molecular weight is preferably from about 30,000 to about 50,000.

The ratio is desirably from about 2.0 to about 2.3 and with 60 the diameter difference being from about 4 to about 12, the ratio is preferably from about 2.0 to about 2.3.

This formulation has been found to be effective to permit 65 the expansion of the sleeve as necessary to place the sleeve over the mandrel without cracking, wrinkling or contracting during the positioning of the sleeve over the mandrel. This results in a sleeve that provides a suitable exterior surface for the blanket cylinder and is dependably installable on the

blanket cylinder. The very high stress on the exterior coating due to the mounting and demounting activities during the manufacturing, testing and usage of such sleeves is readily accomplished without undesirable cracking, wrinkling, deformation or other damage to the exterior coating with the ceramer coating of the present invention.

While the present invention has been described by reference to certain of its preferred embodiments, it is pointed out that the embodiments described are illustrative rather than limiting in nature and that many variations and modifications are possible within the scope of the present invention. Many such variations and modifications may be considered obvious and desirable by those skilled in the art based upon a review of the foregoing description of preferred embodiments.

What is claimed is:

1. A method for producing a polymer sleeve for mounting on a mandrel to form a blanket cylinder for use in an electrophotographic process, the method comprising the steps of:

- a. producing a sleeve having a sidewall of a polymer selected from the group consisting of thermoplastic, thermoset and elastomeric polymers, rigid polyurethanes and blends thereof, the sleeve having an inner diameter from about 1 to about 20 percent less than the outer diameter of the mandrel; and
- b. coating the sleeve with an outer coating comprising a ceramer containing polyurethane and tetraethoxyorthosilicate, the polyurethane having a molecular weight from about 20,000 to about 80,000 with the polyurethane and the tetraethoxyorthosilicate being present in a weight ratio from about 1.8 to about 2.3.

2. The method of claim 1 wherein the sidewall of the sleeve is a rigid polyurethane.

3. The method of claim 1 wherein the molecular weight is from about 30,000 to about 50,000.

4. The method of claim 1 wherein the ratio is from about 2.0 to about 2.3.

5. The method of claim 1 wherein the inner diameter of the sleeve is from about 4 to about 12 percent less than the outer diameter of the mandrel.

6. The method of claim 5 wherein the ratio is from about 2.0 to about 2.3.

7. The method of claim 5 wherein the molecular weight is from about 30,000 to about 50,000.

8. The method of claim 1 wherein the sleeve has a wall thickness from about 1 to about 20 mm.

9. In a method for producing a sleeve for use on a mandrel to produce a blanket cylinder for use in an electrophoto-

graphic process, the sleeve consisting essentially of a sleeve of a polymer selected from the group consisting of thermoplastic, thermoset and elastomeric polymers, rigid polyurethanes and blends thereof and a ceramer coating comprising a polyurethane and tetraethoxyorthosilicate, the sleeve having an inner diameter from about 1 to about 20 percent less than the outer diameter of the mandrel, the improvement comprising adjusting the molecular weight of the polyurethane to from about 20,000 to about 80,000 and adjusting the weight ratio between the polyurethane and the tetraethoxyorthosilicate to from about 1.8 to about 2.3.

10. The method of claim 9 wherein the ratio is from about 2.0 to about 2.3.

11. The method of claim 9 wherein the molecular weight is from about 30,000 to about 50,000.

12. The improvement of claim 9 wherein the inner diameter of the sleeve is from about 4 to about 12 percent smaller than the outer diameter of the mandrel.

13. The method of claim 12 wherein the ratio is from about 2.0 to about 2.3.

14. The method of claim 12 wherein the molecular weight is from about 30,000 to about 50,000.

15. A sleeve adapted to fit over a mandrel to form a blanket cylinder for use in an electrophotographic process, the sleeve comprising:

- a. a sleeve having a sidewall of a polymer selected from the group consisting of thermoplastic, thermoset and elastomeric polymers, rigid polyurethanes and blends thereof, the sleeve having an inner diameter from about 1 to about 20 percent less than the outer diameter of the mandrel; and
- b. an outer coating comprising a ceramer containing a polyurethane and tetraethoxyorthosilicate, the polyurethane having a molecular weight from about 20,000 to about 80,000 with the polyurethane and the tetraethoxyorthosilicate being present in a weight ratio from about 1.8 to about 2.3.

16. The sleeve of claim 15 wherein the sidewall of the sleeve is a rigid polyurethane.

17. The sleeve of claim 15 wherein the molecular weight is from about 30,000 to about 50,000.

18. The sleeve of claim 15 wherein the ratio is from about 2.0 to about 2.3.

19. The sleeve of claim 15 wherein the sleeve has a wall thickness from about 1 to about 20 mm.

\* \* \* \* \*